

Sept. 8, 1936.

J. A. JEFFERY

2,053,369

SPARK PLUG AND METHOD OF MAKING THE SAME

Filed June 24, 1931

*Fig. 1*



*Fig. 2*



*Fig. 3*



*Fig. 4*



Inventor

JOSEPH A. JEFFERY

By

Owen & Owen

Attorneys

## UNITED STATES PATENT OFFICE

2,053,369

SPARK PLUG AND METHOD OF  
MAKING THE SAME

Joseph A. Jeffery, Detroit, Mich., assignor, by  
mesne assignments, to Champion Spark Plug  
Company, Toledo, Ohio, a corporation of Dela-  
ware

Application June 24, 1931, Serial No. 546,557

9 Claims. (Cl. 123—169)

This invention relates to an improvement in  
spark plugs.

The object of the invention is to produce a  
spark plug which will have an insulating mem-  
ber, at least that portion of which is exposed to  
the flame of an internal combustion engine being  
composed of a material which has high resistance  
to chemical reaction with hot gases generally  
found in the combustion chamber of an internal  
10 combustion engine; having high refractory qual-  
ities, high heat conductivity, high heat expansion  
and a high, hot dielectric, and being also dense  
and substantially impermeable to gases. A par-  
ticular object is to guard against the deleterious  
15 results of the fluxing action on the glaze of usual  
spark plugs which is caused by lead compounds  
deposited on the plugs when ethyl gas is used.

The objects of the invention are obtained by  
making at least a portion of the spark plug, that  
20 is exposed to the flames of an internal combus-  
tion engine, from a composition consisting sub-  
stantially of magnesium oxid. Details of the in-  
vention will appear as the description proceeds.

In the drawing, Figure 1 represents a longi-  
25 tudinal section through one form of the improved  
spark plug where the insulating member is made  
in one piece; Fig. 2 is a similar longitudinal sec-  
tion through a plug where the exposed tip of the  
spark plug insulator is made from a different ma-  
30 terial from that composing the outer part of the  
insulator; Fig. 3 is a section similar to Fig. 2,  
but showing a different form of joint between the  
two parts of the insulator; and Fig. 4 is a section  
similar to Fig. 1, but showing a two part core and  
35 a two part insulator.

The construction shown in Fig. 1 comprises an  
insulating member 10 which has extending there-  
40 through an electrode 11. Surrounding the in-  
sulator there is the usual member 12 adapted to  
be screwed into a threaded opening in the cyl-  
inder of an internal combustion engine. The in-  
sulator body is provided with a shoulder 13, the  
45 lower side of which rests upon a packing 14 inter-  
posed between it and a shoulder 15 of casing 12.  
A threaded sleeve 16 screws into the upper end of  
member 12 and compresses a packing 17 against  
the upper side of shoulder 13. Electrode 18 ex-  
50 tends from the lower end of member 12 to spark-  
ing relation with the lower end of electrode 11.

The construction above described is old so far  
as the shape and relation of the various parts is  
concerned, the novelty lying in the composition of  
the insulator 10, which is substantially all mag-  
55 nesium oxid.

It is almost impossible to melt magnesium oxid

so as to cast it with known appliances. It has  
been discovered, however, that granulated mag-  
nesium oxid, especially if the granules are of  
selected sizes so as to pack to the best possible  
advantage, can be pressed into shape and then  
5 sintered sufficiently to form a dense body sub-  
stantially impermeable to gases and having all  
of the qualities enumerated above as desirable in  
the insulating member of a spark plug. It is  
preferable to form the body of graduated sizes  
10 of granules and press it by the dry pressing meth-  
od under high pressure, so as to pack the particles  
as densely and in as intimate relation as possible  
before the firing action.

It has been found that a very small amount  
15 of oxid of cobalt or chromium oxid, Cr<sub>2</sub>O<sub>3</sub>, added  
to the magnesium oxid, reduces the necessary  
temperature for sintering materially, without in-  
juring the qualities of the resultant body, and  
while still leaving the product exceedingly re-  
fractory so that no temperature to which it is  
20 subjected in an internal combustion engine is  
injurious thereto. About one-tenth of one per  
cent of cobalt oxid has been used, and as an  
alternative the same amount of chromium oxid,  
25 this small trace of either of these oxides being suffi-  
cient to lower the sintering temperature of the  
magnesium oxid to a material extent. Other  
basic oxides having a similar effect may be used.

A body made in the above described manner  
30 produces a close knit and strong body when fired  
in a Dressler kiln to cone 17, but small pores  
still remain in the body so that it is somewhat  
permeable to gases. A very satisfactory and  
35 practically impermeable core has been formed  
by sintering the body, a temperature of at least  
1650° C. being required.

Figure 2 discloses a spark plug core similar  
40 to that shown in Fig. 1 except that it is made  
in two parts.

In the insulator body shown in Fig. 2 there  
is a tip 20 formed of approximately pure mag-  
nesium oxid, as described above. The lower  
45 end of this part 20 is that portion of the in-  
sulator body exposed directly to the flame of the  
gases ignited by the spark of the plug and,  
therefore, it is subjected to the highest heat  
conditions.

The upper end 21 of the insulator body is  
not subjected to as high temperature as the low-  
50 er end 20, and therefore, may be made of a  
suitable porcelain or other material not hav-  
ing as high insulating qualities under extreme-  
ly high temperatures as magnesium oxid pos-  
sesses. The two parts of the insulator may be

united by a suitable refractory bond 22, which should also have a fairly high hot dielectric, to avoid the striking of the spark from the central electrode 11 through this bond to the shell 12.

- 5 In Fig. 3 there is shown a core similar to that shown in Fig. 2 except that the upper end of portion 20<sup>b</sup> is roughly conical, with ridges 23 thereon, while the lower end of portion 21<sup>b</sup> is provided with a socket 24 having grooves 25 therein so that refractory bond 22<sup>b</sup> will securely unite the two parts. The conical arrangement of the joint is desirable where the bond is not as good an insulator as other portions of the core, since this arrangement lengthens the path 10 through the bond. This arrangement also provides for holding the two parts of the core in accurate alinement, so that the central passages for the electrode remain in alinement.

The form shown in Fig. 4 is similar to that 20 shown in Fig. 2, with minor differences. The shell etc., are the same as shown in Fig. 1, and are accordingly designated by the same numerals. The inner end 20<sup>c</sup> of the insulator is made of magnesium oxide and has in its upper end a socket 26 into which there fits an extension 27 from the lower end of the upper part 21<sup>c</sup> of the insulator. An electrode 28 projects downward through part 20<sup>c</sup>, and has a head 29 fitting in the bottom of socket 26. The electrode 30 may be secured in place at 30 by screw threads or a suitable bond or both. The upper portion 21<sup>c</sup> of the insulator has an electrode 31 extending downward therethrough and terminating in a head 32 adapted to rest upon head 29. Electrode 31 may be held in place by a nut 33 on its screw threaded upper end.

In this construction the two parts of the insulator carry their respective portions of the electrode, and so may be handled and replaced separately. They may be held together by shoulder 15 and collar 16 of the shell.

The described method of making the insulator body renders it convenient where it is desired to make the entire body of magnesium oxide, and this is the preferred construction, although the magnesium oxide composition is particularly necessary only in the more exposed portion of the body.

It will be readily understood that the shape 50 of the insulator body may be changed as desired for various reasons, and that, where a two part body is formed, the exposed part may be held in position by other means than those

disclosed, the essential feature of this invention being the composition and method of making the exposed part of the insulator body.

In the specification and claims the term "approximately pure magnesium oxide" is intended 5 to cover a product which is not absolutely pure, but which is as pure as any that was available upon the market commercially at the time this application was filed.

What I claim is:

1. A spark plug comprising an insulating body having the portion at the sparking end of the plug composed of approximately pure sintered magnesium oxid. 10

2. A spark plug comprising an insulating body having the portion at the sparking end of the plug composed of approximately pure sintered magnesium oxid substantially impermeable to gases. 15

3. A spark plug comprising a unitary self-sustaining insulator body made entirely of substantially pure magnesium oxid. 20

4. A spark plug comprising a self-sustaining insulating body composed of upwards of 99% magnesium oxid and less than 1% of impurities. 25

5. A spark plug comprising a self-sustaining insulating body composed of upwards of 99% magnesium oxid and less than 1% of impurities and sintered into a body substantially impermeable to gases. 30

6. A spark plug comprising a self-sustaining insulating body composed of upwards of 99% magnesium oxid and a trace of a refractory oxid which lowers the sintering temperature of magnesium oxid without materially affecting the insulating qualities thereof. 35

7. A spark plug comprising a self-sustaining insulating body composed of upwards of 99% of magnesium oxid and a fraction of 1% of cobalt oxid. 40

8. A spark plug comprising a self-sustaining insulating body composed of upwards of 99% of magnesium oxid and a fraction of 1% of chromium oxid. 45

9. A spark plug comprising an insulating core having a shoulder around its middle and a shell pressing against the two sides of the shoulder, the core being divided into two separable parts across the shoulder, so that the shell presses the two parts of the core against each other, the inner part of the core being of magnesium oxide. 50

JOSEPH A. JEFFERY.